

## UNITED STATES PATENT OFFICE.

HARRY W. MORSE, OF STANFORD UNIVERSITY, CALIFORNIA, ASSIGNOR TO COMPAGNIE DU BOLEO, OF SAN FRANCISCO, CALIFORNIA, A CORPORATION OF FRANCE.

## FLOTATION OF ORES.

No Drawing.

Application filed July 29, 1925. Serial No. 46,860.

This invention relates to the recovery of copper and other metals from ores by the flotation process and the main object of the invention is to provide a process which will be capable of successful operations upon certain ores with high recovery and low cost.

My process consists essentially in subjecting the ore to flotation operation in the presence of a flotation agent consisting of a xanthate of an alkali metal together with an alkali metal chloride, for example sodium chloride, or material containing sodium chloride, such as sea water.

I have applied my invention successfully to the recovery of copper from copper ores containing about 4% copper mainly in the form of sulphides, but with about .1 to .4% of oxides and with a gangue consisting mainly of a clay-like mass. The sulphide constituent of the ore comprises chalcocite, bornite, and covellite, and in addition to the sulphide and oxide content, there is a little native copper present. The ore in question is produced from the below named mines of the Compagnie du Boleo in Baja California, Mexico, and is not amenable to flotation by the use of the usual flotation agents, or by the use of sodium or potassium xanthate without the use of sodium chloride.

In carrying out my process the ore is first crushed and ground to bring it to a suitable state of division, say 80 mesh, or finer, and to the pulp containing the finely ground ore and water is added a flotation agent consisting of about 0.2 to 0.4% of sodium or potassium xanthate together with a suitable amount of sodium chloride. Such suitable amount may be obtained by using sea water as a liquid which is ground with the ore to form the pulp but in any case it is desirable to have from 2% to 4% of sodium chloride present in the water of the pulp during the flotation operation, and in case sea water is not available this amount of sodium chloride may be added to the water in the pulp, either before, during, or after the grinding. No other reagent, such as a frothing agent, need be present during the flotation operation. The flotation may be ef-

fected in any suitable flotation machine, either agitating or aeration type, and the copper values recovered by flotation in the usual manner in such operations. Tests made on ore of the character above described have given the following results:

55

## Montado.

| Percentage recovery of copper. | Percentage Cu in first concentrates |
|--------------------------------|-------------------------------------|
| 82.5                           | 39.00                               |
| 81.0                           | 28.50                               |
| 80.0                           | 35.30                               |
| 81.2 Average                   | 31.3 Average                        |

60

## Margarita.

| Percentage recovery of copper. | Percentage Cu in first concentrates. |
|--------------------------------|--------------------------------------|
| 87.0                           | 39.8                                 |
| 88.0                           | 40.1                                 |
| 88.0                           | 41.0                                 |
| 88.0                           | 41.1                                 |
| 90.0                           | 42.8                                 |
| 87.0                           | 32.4                                 |
| 88.0 Average                   | 39.5 Average                         |

65

## Santa Rita.

| Percentage recovery of copper. | Percentage Cu in first concentrates. |
|--------------------------------|--------------------------------------|
| 83.0                           | 32.5                                 |
| 85.0                           | 36.3                                 |
| 83.0                           | 33.1                                 |
| 83.7 Average                   | 34.8 Average                         |

70

75

80

I have also applied my process successfully to flotation of a lead zinc ore, sodium xanthate in the presence of salt in solution enabling decided selective flotation of the lead sulphide from zinc sulphide. The proportions of xanthate and sodium chloride in these cases is substantially the same as in the flotation of ore from the mines of the above-named Compagnie du Boleo.

## What I claim:

1. The process of recovering metal from its ores which consists in subjecting the pulp containing the ore to a froth flotation operation in the presence of a flotation agent con-

sisting of an alkali metal xanthate together with an alkali metal chloride.

2. The process as set forth in claim 1 in which the flotation agent consists of an alkali metal xanthate together with sodium chloride.

3. The process of recovering copper from

its ores which consists in subjecting the pulp containing the ore and sea water together with an alkali metal xanthate to a froth 10 flotation operation.

In testimony whereof I have hereunto subscribed my name this 17th day of June, 1925.

HARRY W. MORSE.